

E. W. McMULLEN.

METAL COATING.

APPLICATION FILED FEB. 11, 1918.

1,268,987.

Patented June 11, 1918.



Witnesses:

Arthur H. Carlson

Robert H. Ulmer

Inventor  
Earle W. McMullen  
By  
Offield Towle Graves & Offield  
Attn.

# UNITED STATES PATENT OFFICE.

EARLE W. McMULLEN, OF KENOSHA, WISCONSIN, ASSIGNOR TO SIMMONS COMPANY, OF KENOSHA, WISCONSIN, A CORPORATION OF DELAWARE.

## METAL COATING.

1,268,987.

Specification of Letters Patent. Patented June 11, 1918.

Application filed February 11, 1918. Serial No. 216,581.

To all whom it may concern:

Be it known that I, EARLE W. McMULLEN, a citizen of the United States, residing in the city of Kenosha, county of Kenosha, 5 and State of Wisconsin, have invented certain new and useful Improvements in Metal Coatings, of which the following is a specification.

My invention relates to improvements in 10 metal coatings and has particular reference to an ornamental finish for steel or other ferrous metal.

The object of the invention is to provide 15 for steel articles a practically indestructible coating, or finish, which shall possess sanitary and ornamental properties and characteristics to a high degree, while at the same time having great durability and mechanical strength and the maximum adhesive effect.

20 My invention briefly involves the covering of steel or other ferrous metal with an electrolytic deposit of zinc and subsequently applying, by spraying or otherwise, to the top of said coating a finishing coat of tough lacquer or analogous material.

The drawing shows a piece of ferrous metal coated according to my process.

During recent years liquid finishes, generally known in the trade as lacquers have 30 been developed and utilized to a considerable extent for the purpose of coating metal articles and with considerable success in so far as they may have been used upon non-ferrous or non-oxidizable metals such as 35 brass, copper and the like. However, so far as I am informed, no practical lacquer has, up to the present, been successfully developed for use directly upon the outer surface of an article made of a ferrous metal 40 which, when in the proper finished condition, does not furnish a foundation to which lacquer will stick with any degree of certainty. Also it has been found that when lacquer is applied directly to a steel surface 45 it does not adequately protect the steel against rust due to the oxidizing effect of the atmosphere.

I have discovered that certain grades of 50 lacquer and particularly that kind of lacquer which has a cellulose or celluloid base can be successfully applied to steel, if the latter be first coated electrically with a non-ferrous metal such as zinc. This discovery was made by me after numerous attempts to 55 secure the same result by first coating metal

parts with the zinc by means of the "hot process," that is to say by dipping the article into a bath of molten zinc. These attempts of mine to lacquer hot galvanized steel parts were, however, uniformly unsuccessful for the reason, I believe, in the light of my present knowledge, that a hot galvanized coating is too smooth to provide the necessary adhesive effect. On the other hand I have discovered that the surface of 60 a steel article to which there has been applied an electrolytic deposit of zinc furnishes an admirable foundation for the lacquer for the reason that the surface of said deposit when examined under a microscope 70 is found to be of a uniform crystalline texture to which the lacquer adheres with the greatest tenacity.

Although it is possible that other types 75 of lacquer may be employed in practising my invention, I prefer to use a lacquer of the cellulose group, i. e., a lacquer derived from cellulose. The one with which I have secured the best results is the celluloid lacquer.

No special apparatus is required for carrying out my invention. As successfully carried out the steel article to be coated is galvanized electrically by the "cold process" in the same manner as any ordinary 85 electroplating process, after which the article is washed and dried in the usual manner and when dry is sprayed with the lacquer by means of a suitable air brush. When dry the lacquer coating is strongly adherent 90 to the surface of the metal and will not flake off or crack even though the surface of the metal be very seriously disfigured or otherwise distorted out of its original shape. This feature is of inestimable value in the 95 case of metal bedsteads or other furniture constructed of relatively thin steel sheets or tubing such as is now rapidly becoming the best modern practice in metal furniture construction.

100 My improved coating has the additional advantage that in the event the surface of the lacquer is accidentally removed by abrasion, or otherwise, the surface of the steel does not oxidize and rust because it is 105 protected by the zinc coating beneath the lacquer.

110 It should be understood that my invention is not confined to transparent lacquer but may be used for producing all kinds of lac-

quer finish according to present day lacquering practice.

I claim:—

- 5 1. The improvement in the art of coating steel or other ferrous metal which consists in electrolytically depositing a coating of zinc upon the surface of the metal and subsequently covering the said deposit with lacquer.
- 10 2. The improvement in the art of beautifying and protecting a steel surface which consists in electrolytically depositing a coat-

ing of zinc upon the said surface and subsequently coating the deposit with a cellulose lacquer.

3. As a new article of manufacture, a lacquered ferrous article provided with an intermediate electrolytic zinc deposit under the lacquer coating.

4. As a new article of manufacture, a steel part coated electrolytically with zinc deposit, and having an outer coat of cellulose lacquer covering said deposit.

EARLE W. McMULLEN.